

F. J. LYSTER,  
CONCENTRATION OF ORES,  
APPLICATION FILED JULY 14, 1915,

1,203,373.

Patented Oct. 31, 1916.

2 SHEETS—SHEET 1.



Fig. 1.

Inventor:  
Henry James Lyster  
By Henry W. Williams  
Attorney.

F. J. LYSTER.  
CONCENTRATION OF ORES.  
APPLICATION FILED JULY 14, 1915.

1,203,373.

Patented Oct. 31, 1916.

2 SHEETS—SHEET 2.



Inventor  
Fleury James Lyster  
By Kenny D. Williams  
Attorney.

# UNITED STATES PATENT OFFICE.

FLEURY JAMES LYSTER, OF BROKEN HILL, NEW SOUTH WALES, AUSTRALIA, ASSIGNOR  
BY MESNE ASSIGNMENTS, TO MINERALS SEPARATION AMERICAN SYNDICATE (1913)  
LIMITED, OF LONDON, ENGLAND.

## CONCENTRATION OF ORES.

1,203,373.

Specification of Letters Patent. Patented Oct. 31, 1916.

Original application filed May 8, 1913, Serial No. 766,346. Divided and this application filed July 14, 1915.  
Serial No. 39,927.

To all whom it may concern:

Be it known that I, FLEURY JAMES LYSTER, subject of the King of Great Britain and Ireland, residing at Broken Hill, in the 5 State of New South Wales, Commonwealth of Australia, have invented certain new and useful Improvements in the Concentration of Ores, of which the following is a specification, reference being had therein to the accompanying drawings, forming part thereof.

This invention relates to improvements in the concentration of ores and is particularly applicable to the separation of mixed zinc and lead sulfid ores, and this application 15 is a division of my application filed May 8, 1913, Serial No. 766,346.

The object of this invention is to separate metalliferous portions of an ore such, for example, as the sulfid of lead (galena) from 20 other portions of the ore, and more particularly to effect a differential or selective flotation in the treatment of mixed zinc and lead sulfid ores, to wit: the separation of lead sulfid (galena) from zinc sulfid 25 (blende), obtaining a product relatively rich in lead on the one hand, and a zinc product relatively low in lead on the other hand.

I have discovered that sulfid of lead (galena) may be separated from sulfid of 30 zinc (blende) without any preliminary treatment by subjecting the ore or metalliferous materials to a flotation separation treatment at a low temperature with eucalyptus oil or other frothing agent and 35 with agitation or aeration in an alkaline solution containing, for example carbonate of sodium.

The suitability of any given substance in 40 an alkaline solution can be easily determined by a laboratory test as hereinafter described.

In carrying this process into effect a plant similar to that employed in and common to agitation froth processes may be employed.

45 I have shown in the accompanying drawings two forms of apparatus adapted for carrying out my process.

Figure 1 is a longitudinal elevation and Fig. 2 a cross-section of a unit with the 50 supply devices in elevation, and Fig. 3 is a sectional elevation of an apparatus suitable for testing.

I will now describe my process as carried out in the apparatus shown in Figs. 1 and 2.

The ore is first ground to a suitable degree 55 of fineness (preferably to slimes so that the different metallic sulfid particles are disassociated from each other). This finely ground ore with its accompanying circuit water (which is a solution such as hereinbefore described) is led into a settler or thickener A to remove excess water. The thickened pulp is then led into a vessel B, from which it passes to the first centrifugal pump C<sup>1</sup> of the series C<sup>1</sup>, C<sup>2</sup>, C<sup>3</sup>, C<sup>4</sup>, C<sup>5</sup>, C<sup>6</sup>. 60 These centrifugal pumps are each connected to the individual members of a corresponding series of separating boxes D<sup>1</sup>, D<sup>2</sup>, D<sup>3</sup>, D<sup>4</sup>, D<sup>5</sup>, D<sup>6</sup>. These centrifugal pumps act as agitators or mixers and means are provided 70 (such as an inlet pipe E) for feeding in the requisite amount of eucalyptus oil or other frothing agent, about 2 lbs. per ton of material treated, as well as the requisite amount of air (such as by a tap F) into the 75 suction pipe G<sup>1</sup> thereof, which is connected to the feed vessel B. The centrifugal pump C<sup>1</sup> draws in pulp, air, and frothing agent, and produces an intimate mixture which is discharged through the outlet pipe H to the 80 separator box D<sup>1</sup>, the delivery of the pump being controlled by the admission of air by the tap F. The particles of lead sulfid (galena) are found to rise to the top of the separator box D<sup>1</sup>, where an inverted pyramid J<sup>1</sup> diverts the froth toward the discharge lip or launder K<sup>1</sup>, from which it flows to the receptacle for settling and collecting the lead concentrate. The particles which do not rise or float, together with the 85 balance of the water, sink to the bottom of the box D<sup>1</sup> and are there withdrawn by the outlet pipe L<sup>1</sup> which is connected to the suction pipe G<sup>2</sup> of the next pump C<sup>2</sup> of the series, and the operation is repeated, the 90 residues of one separator box D<sup>1</sup> passing to the centrifugal pump C of the next in series.

In the plant illustrated in the accompanying drawings there are six separator boxes and their attendant pumps, which comprise 100 one series or unit, but it will be understood that this number is dependent upon the proportion of mineral contained in the ore and the degree of agitation and aeration re-

quired, the repetition of the operations being carried on until the grade of the concentrates becomes too low in lead and the zinc begins to appear therein. The temperature I prefer is below 100° Fahr. That is to say, the operation is conducted at the ordinary temperature and no extraneous heat is utilized.

I have observed in working the process for the selective flotation of lead sulfids from what are known as calcitic slimes at Broken Hill that an excessive alkalinity tends to retard the selective flotation of the lead sulfid particles. Therefore when the process is used with this ore for this purpose the solution should be only slightly alkaline, but sufficient to respond to the well known methyl orange test.

The suitability of the substances hereinbefore indicated and the proportion thereof to the solution and the degree and duration of agitation or aeration of the material treated can be determined in a laboratory test which may be conducted as follows in an apparatus such as is illustrated in Fig. 3 of the accompanying drawings: This apparatus comprises an agitating or mixing vessel N having a rotating impeller O, a separating box P on the side thereof connected to the mixer by a passage R and by a flexible hose pipe S at the bottom. In carrying out a test the mixing vessel N contains the solution which corresponds with the circuit water of the working plant, and eucalyptus or other frothing agent is then added in measured quantities. The impeller O is then rotated at about 1700 revolutions per minute and a charge of about 448 grammes of ore is fed in. Sufficient solution is added to fill the separating box P to the level of its discharge lip. The agitated pulp is forced through the passage R into the separating box P and the float or froth rising to the surface is skimmed off over the lip. The pulp is continuously circulated by being drawn from the bottom of the box P by the pipe S back into the mixer N by the action of the impeller O. The flotation is continued until the float or froth is noticed by observation to become lower in lead and the zinc begins to appear therein. The appearance of the concentrate being skimmed off over the lip of the separating box will indicate the duration of agitation necessary to obtain a good concentrate combined with a good recovery, while experience will indicate the amount of frothing agent necessary, and further quantities may be added at intervals as found necessary. The residue is run off from the bottom of the machine by disconnecting the flexible hose or pipe S. Repeated trials with different solutions and with different strengths will indicate what is best suited to the particular ore under treatment. The ascer-

tained duration of agitation and aeration will govern the number of separator boxes which will be necessary in the working plant when that hereinbefore described is used.

I have found that in obtaining a selective separation of the lead sulfids from the zinc sulfids in the ore heretofore referred to, known as calcitic slimes at Broken Hill, to which my process is peculiarly well suited, averaging about eleven per cent. (11%) of zinc and about thirteen per cent. (13%) of lead, and using about from two (2) to five (5) lbs. of eucalyptus per ton, I have obtained good results with a solution of sodium carbonate in the proportion of 500 grains per gallon. I have also obtained good results with a solution of sodium bicarbonate in the proportion of 600 grains per gallon.

In another modification of the above procedure I have used calcium chlorid, 300 grains per gallon, with calcium hydrate, 3.6 grains per gallon, and in another modification have used calcium nitrate, 300 grains per gallon, with calcium hydrate, 18 grains per gallon.

I have further discovered that the residues obtained as before described, containing the bulk of the zinc sulfids may be further treated by flotation separation to produce a concentrate rich in zinc by first dewatering and thickening the pulp and then submitting it to a repetition of the flotation separation, using, however, sufficient water in lieu of the solution previously employed, or by further continuing the process hereinbefore described, after the recovery of the lead sulfids (galena) in a separate de-zincing unit until the zinc sulfids (blende) appear upon the surface of the solution and are carried over into the launder hereinbefore mentioned. In operation I prefer the former to the latter method for the recovery of the zinc sulfids (blende). In this way a zinc concentrate may be obtained and thereby both the lead sulfids and zinc sulfids recovered in separate products by flotation separation without recourse to separation by gravitation or tables or vanners as heretofore.

I claim:—

1. A process of concentrating ores which consists in agitating and aerating an ore pulp containing in solution an alkaline selectivity-modifying agent and containing a small proportion of a frothing agent, so as to obtain a froth of concentrates, the solution being alkaline during separation and separating the froth.

2. A process of concentrating ores which consists in agitating and aerating an ore pulp containing in solution a salt of a mineral acid having an alkaline reaction and containing a small proportion of a frothing agent, so as to obtain a froth of concentrates, the solution being alkaline during separation and separating the froth.

3. A process of concentrating ores which consists in agitating and aerating an ore pulp containing sodium carbonate in solution and containing a small proportion of a 5 frothing agent, so as to obtain a froth of concentrates, the solution being alkaline during separation and separating the froth.
4. A process for the separation of lead sulfids (galena) from zinc sulfids (blende) 10 in ores containing mixed lead and zinc sulfids which consists in subjecting the said ores to the agitation froth process by agitating them with a frothing agent in an alkaline solution, thereby separating the lead sulfids 15 from the zinc sulfids.
5. A process for the separation of lead sulfids (galena) from zinc sulfids (blende) in ores containing mixed lead and zinc sulfids which consists in subjecting the said 20 ores to the agitation froth process by agitating them with a frothing agent in an alkaline solution containing a compound of an alkaline metal, thereby separating the lead sulfids from the zinc sulfids.
6. A process for the separation of lead sulfids (galena) from zinc sulfids (blende) in ores containing mixed lead and zinc sulfids which consists in subjecting the said ores 25 to the agitation froth process by agitating them with a frothing agent in an alkaline solution containing sodium carbonate, thereby separating the lead sulfids from the zinc sulfids.
7. A process for the separation of lead sulfids (galena) from zinc sulfids (blende) in ores containing mixed lead and zinc sulfids, which consists in subjecting the said ores to the agitation froth process by agitating 30 them with a frothing agent in an alkaline solution, thereby obtaining a concentrate relatively rich in lead, and in submitting the residues to a dewatering and thickening operation and finally subjecting the same to a repetition of the agitation froth process with fresh water in lieu of the solutions previously employed, thereby obtaining a concentrate relatively rich in zinc.
8. A process for the separation of lead sulfids (galena) from zinc sulfids (blende) in 35 ores containing mixed lead and zinc sulfids which consists in subjecting the said ores to the agitation froth process by agitating them with a frothing agent in an alkaline solution containing a compound of an alkaline metal, thereby obtaining a concentrate relatively rich in lead, and in submitting the residues to further agitation, thereby obtaining a concentrate relatively rich in zinc.
9. A process for the separation of lead sulfids (galena) from zinc sulfids (blende) in ores containing mixed lead and zinc sulfids 40 which consists in subjecting the said ores to the agitation froth process by agitating them with a frothing agent in an alkaline solution containing sodium carbonate, thereby obtaining a concentrate relatively rich in lead, and in submitting the residues to a dewatering and thickening operation and finally subjecting the same to a repetition of the agitation froth process with fresh water in lieu of the solutions previously employed, thereby obtaining a concentrate relatively rich in zinc.
10. A process for the separation of lead sulfids (galena) from zinc sulfids (blende) in ores containing mixed lead and zinc sulfids 45 by subjecting the said ores to the agitation froth process by agitating them with a frothing agent in an alkaline solution, thereby obtaining a concentrate relatively rich in lead and in submitting the residues to further agitation, thereby obtaining a concentrate relatively rich in zinc.
11. A process for the separation of lead sulfids (galena) from zinc sulfids (blende) in ores containing mixed lead and zinc sulfids, by subjecting the said ores to the agitation froth process by agitating them with a frothing agent in an alkaline solution containing a compound of an alkaline metal, thereby obtaining a concentrate relatively 50 rich in lead and in submitting the residues to further agitation, thereby obtaining a concentrate relatively rich in zinc.
12. A process for the separation of lead sulfids (galena) from zinc sulfids (blende) in ores containing mixed lead and zinc sulfids, by subjecting the said ores to the agitation froth process by agitating them with a frothing agent in an alkaline solution containing sodium carbonate, thereby obtaining a concentrate relatively rich in lead and in 55 submitting the residues to further agitation, thereby obtaining a concentrate relatively rich in zinc.
- In testimony whereof I have affixed my 110 signature in presence of two witnesses.
- FLEURY JAMES LYSTER,
- Witnesses:
- ARTHUR GORE COLLISON,  
LESLIE HERBERT BROADBENT.